

## UNITED STATES PATENT OFFICE.

JOHN F. EDWARDS, OF WARREN, ARKANSAS.

## COMPOUND FOR TEMPERING TOOLS AND TOOL STEEL.

No Drawing.

Application filed December 13, 1926. Serial No. 154,657.

My present invention relates to a special bath which I have found especially effective in treating tool steel. I have found that the solution of certain chemicals namely glycerine, spirits of nitre, ammonia, sal-ammoniac, sulphate of zinc and alum in certain defined proportions which has heretofore been for carbureting steel will produce an efficient quenching bath if certain other ingredients are added to the bath. However, the compound, if used in the density heretobefore employed for carburetting, no satisfactory results are obtained in quenching tool steel. I have found however by greatly diluting the solution this compound is somewhat effective in tempering but by the addition of such other ingredients to these compounds and by treating the tool in a very dilute bath steel of a high carbon content may be hardened by the usual quenching procedure to effect a fine granular texture containing the various carbides in proper proportion to render the tool effective and durable.

A tool treated by quenching in a bath containing the ingredients above noted and a density used for carburetting is too soft even when sulphate of copper is added to the bath as a hardener. I have discovered that the compound if used in a very dilute form gives better results, but with the addition of other ingredients which I have successfully added I find that greatly improved results are obtained. The solution I have referred to as used for carburetting contains three ounces of commercial glycerine, one and a half ounces of spirit of nitre, one and one half ounces of aqua ammonia, two ounces of chloride of ammonia, one and one half ounces of sulphate of zinc, one and one half ounces of sulphate of alumina and ammonia or aluminum ammonium alum dissolved in a half gallon of water.

A bath of these materials if used in the density employed for carburetting applied in hardening tool steel articles is not at all effective leaving them too soft. If, however, the bath is diluted the hardening effect begins to show and when it reaches the very high degree of dilution taking only two ounces of the mixture above described to a gallon of water better results in hardening

may be effected. I have found now, however, that by adding to a solution of this kind highly diluted one ounce of pure glycerine, one half ounce of table salt, one eighth ounce of copper sulphate and one half ounce of alum that the best results will be obtained. I have given the formula employed in the carburetting process to distinguish between a bath for raising the carbon content and a formula suitable for tempering tool steel which already has a high carbon content. According to my experience the quality of glycerine is important, it being essential to best results to employ pure glycerine. Some of the ingredients may be reduced or omitted but I have found that the addition of table salt and copper sulphate in substantial proportion is important to successful results.

My invention therefore consists in a solution or bath for quenching tool steel consisting of a very dilute solution containing glycerine, nitre, ammonia, sal-ammoniac, alum and zinc sulphate to which is added common salt, alum and copper sulphate in very much larger proportions for tempering. The implement or tool is brought to a cherry red and immersed in the bath of the dilution described. It is then reheated to a color depending on the temper desired, and chilled in pure water.

Having thus described my invention, what I claim as new and desire to secure by Letters Patent is:

A liquid bath for quenching tool steel, consisting of the following ingredients in the following approximate proportions:

|                                | Approximate<br>metric<br>equivalents. | 90          |
|--------------------------------|---------------------------------------|-------------|
| Glycerin                       | 3 fluid ounces                        | 96 c. c.    |
| Sweet spirit of nitre          | 1½ fluid ounces                       | 48 c. c.    |
| Ammonium chloride              | 1½ ounces                             | 48 gm.      |
| Zinc sulphate                  | 1½ ounces                             | 48 gm.      |
| Aluminum and ammonium sulphate | 1½ ounces                             | 48 gm.      |
| Water                          | 1 gallon                              | 2,000 c. c. |

of the foregoing two fluid ounces is added to one gallon of water containing:

|                        |               |          |
|------------------------|---------------|----------|
| Glycerin               | 1 fluid ounce | 32 c. c. |
| Sodium chloride        | ½ ounce       | 16 gm.   |
| Aluminum ammonium alum | ½ ounce       | 16 gm.   |
| Copper sulphate        | ½ ounce       | 4 gm.    |

In testimony whereof I affix my signature.

JOHN F. EDWARDS.